

# United States Patent Office

2,874,047

Patented Feb. 17, 1959

1

2,874,047

## PHOTOSENSITIVE COMPOSITION

Peter A. van der Meulen, Highland Park, N. J., and Paul B. Gilman, Jr., Rochester, N. Y., assignors to the United States of America as represented by the Secretary of the Air Force

No Drawing. Application November 4, 1957

Serial No. 694,462

9 Claims. (Cl. 96—94)

The present invention relates generally to photosensitive materials and, as illustrated herein, relates more particularly to such materials wherein the heat developed image may be removed and the original photosensitivity of the material will be restored.

Photothermographic material may be differentially modified or decomposed by the action of heat in accordance with previous response to light to produce a visible image. Silver oxalate and mercurous oxalate have been used for the manufacture of photographic layers. These materials, however, have not been entirely satisfactory since they have a relatively low sensitivity to light and hence require relatively long exposures to produce a negative which when developed will have sufficient contrast. Somewhat higher photothermal sensitivity is produced by a coprecipitated mixture of silver and mercurous oxalate. Sensitivity may be still further increased by adding an excess of potassium oxalate. However, such compositions can be used only once since it is not possible to restore light sensitivity to the original layer.

One object of the present invention is to provide a material which is highly sensitive to light and which may be reactivated by a simple process for reuse. To this end, a mercurous iodide-silver iodide mixture is provided which is dispersed in a gelatin solution and coated on a suitable surface. Preferably, and as illustrated, the mixture contains mercurous iodide ( $Hg_2I_2$ ) and silver iodide ( $AgI$ ) wherein the silver iodide comprises from .1 to 90 mole percent of the mixture, since such a ratio provides greater sensitivity over a wider wavelength range.

The present invention will become more apparent from the following description of a method for preparing a mixture of iodides by the use of which highly sensitive photosensitive material is produced. The method of preparing the iodides and the range of mole ratios in which they are to be combined may be varied within wide limits. The reaction temperatures and the reaction time may also be varied within reasonable limits without involving any substantial change in the photosensitivity of the mixture.

The present invention is based broadly on the discovery that mercurous iodide-silver iodide mixtures containing from .1 to 90 mole percent of silver iodide are photosensitive and latent images may be developed either chemically or thermally, after relatively short exposures to light. Generally, the photosensitivity of the mixture varies as the mole percent of silver iodide in the mixture varies.

The present mixture of ingredients may be developed thermally by heating the exposed mixture for four minutes at a temperature of approximately 105° C.

The image developed thermally is stable but it is possible to restore the mixture to its initial photosensitive condition by continued heating at 130° C. for thirty minutes and the mixture therefore is reusable. However, thermal reversal is not possible when the mercurous iodide-silver iodide mixture is chemically developed.

2

An example for preparing a photographic emulsion of mercurous iodide and silver iodide is as follows:

|    |                      |    |      |
|----|----------------------|----|------|
| 5  | A. Potassium iodide  | g  | 6.0  |
|    | Distilled water      | ml | 300  |
| 10 | B. Mercurous nitrate | g  | 11.2 |
|    | 6 N nitric acid      | ml | 10   |
|    | Distilled water      | ml | 400  |
| 15 | C. Silver nitrate    | g  | .46  |
|    | Distilled water      | ml | 100  |
| 20 | D. Potassium iodide  | g  | .40  |
|    | Distilled water      | ml | 100  |
| 25 | E. Gelatin           | g  | 37.5 |
|    | Distilled water      | ml | 150  |

The various materials are dissolved in distilled water in the amounts noted above. The procedures outlined below are carried under darkroom conditions using a red safelight.

20 Solution A is added very slowly and with rapid agitation to Solution B. The resulting precipitate is stirred for two minutes and then washed by decantation with approximately three liters of distilled water.

25 Solution C is added within thirty seconds to rapidly agitated solution D. The resulting silver iodide precipitate is stirred for two minutes and then is added directly to the mercurous iodide-water mixture resulting from the reactions between solutions A and B. The mixed precipitates are stirred for three minutes, washed by decantation and dispersed in solution E at 50° C.

30 The emulsion is then passed through a hand homogenizer and coated on transparent slides formed of suitable clear plastic or glass. The slides are dried overnight and are then ready for use.

35 It is to be noted that the mercurous-iodide and silver iodide mixtures may vary from .1 to 90 mole percent of silver iodide. The best results, however, are obtained when the silver iodide is present in the mixture in 1.0 to 10 mole percent. The above mixtures are highly sensitive to light in the visible range up to approximately 490 millimicrons.

40 After the coated slide has been exposed, the latent image thereon may be thermally developed by placing the properly exposed plate on a heated block emulsion side up at a temperature of 105° C. for a period of four minutes.

45 Chemical development can be carried out in the conventional manner by immersing the exposed plate for two minutes in 1:2 solution of Kodak Dektol.

50 It is apparent that the present invention may be used for making reversible print-out materials for the production of photographs of documents, for the rapid production of reversible negatives or positives by thermal development and for the production of irreversible negatives or positives with chemical development.

55 Having thus described our invention, what we claim as new and desire to secure by Letters Patent of the United States is:

60 1. A photographic element comprising a support, a gelatine carrier, and heat sensitive material carried thereby, said heat sensitive material comprising from 0.1 to 90 mole percent of silver iodide and from 99.9 to 10 mole percent of mercurous iodide.

65 2. A photographic element comprising a support, a gelatine carrier, and heat sensitive material carried thereby, said heat sensitive material comprising from 1.0 to 10 mole percent of silver iodide and from 99 to 90 mole percent of mercurous iodide.

70 3. A photographic element comprising a support and a heat sensitive gelatine layer thereon containing gelatin and light and heat sensitive materials, said materials com-

prising 0.1 to 90 mole percent of silver iodide and from 99.9 to 10 mole percent of mercurous iodide.

4. A photographic element comprising a support and heat sensitive gelatine layer thereon comprising gelatin and light and heat sensitive materials, said materials comprising 0.1 to 90 mole percent of silver iodide and 99.9 to 10 mole percent of mercurous iodide.

5. A method of making a visible image which comprises sensitizing a gelatine layer with light sensitive mixture of .1 to 90 mole percent silver iodide and 10 to 99.9 mole percent of mercurous iodide and heating said layer to a temperature of about 105° C. to produce an image therein.

6. A method of making a visible image which comprises sensitizing a gelatine layer with light sensitive mixture of .1 to 90 mole percent of silver iodide and 10 to 99.9 mole percent of mercurous iodide, exposing said layer to light, and then submitting said layer to a temperature of about 105° C. to develop the latent image therein, and finally submitting said layer to a temperature of about 130° C. to restore the sensitivity of said layer.

7. A method of making a visible image which comprises sensitizing a gelatine layer with a light and heat sensitive mixture of .1 to 90 mole percent of silver iodide and 10 to 99.9 mole percent mercurous iodide, and submitting said layer to heat at a temperature of approxi-

20 mately 105° C. for a period of approximately four minutes to sensitize said layer.

5 8. A method of making a visible image which comprises sensitizing a gelatine layer with a light and heat sensitive mixture of .1 to 90 mole percent of silver iodide and 10 to 99.9 mole percent of mercurous iodide, submitting said layer to heat at a temperature of approximately 105° C. for a period of approximately four minutes to sensitize said layer, and finally heating said layer to a temperature of about 130° C. for a longer period of time to restore the sensitivity of said layer.

10 9. A method of making a visible image which comprises sensitizing a gelatine layer with a light and heat sensitive mixture of .1 to 90 mole percent of silver iodide and 10 to 99.9 mole percent of mercurous iodide, submitting said layer to heat at a temperature of approximately 105° C. for a period of approximately four minutes to sensitize said layer, and finally heating said layer to a temperature of approximately 130° C. for a period of approximately thirty minutes.

#### References Cited in the file of this patent

#### UNITED STATES PATENTS

|           |                            |               |
|-----------|----------------------------|---------------|
| 1,738,530 | Frankenburger et al. ----- | Dec. 10, 1929 |
| 2,700,610 | Suchow et al. -----        | Jan. 25, 1955 |
| 2,728,664 | Carroll et al. -----       | Dec. 27, 1955 |